

Sept. 5, 1967

T. S. CLORAN ET AL  
METHOD FOR PRODUCING COMPACTED ARTICLES HAVING  
LARGE LENGTH TO DIAMETER RATIOS  
Filed Dec. 27, 1966

3,340,055



INVENTORS.  
THOMAS S. CLORAN &  
VERNON R. THOMPSON  
By *Clair L. Muller Jr.*  
Attorney

# United States Patent Office

3,340,055

Patented Sept. 5, 1967

1

3,340,055

## METHOD FOR PRODUCING COMPAKTED ARTICLES HAVING LARGE LENGTH TO DIAMETER RATIOS

Thomas S. Cioran, East Liverpool, Ohio, and Vernon R. Thompson, Pittsburgh, Pa., assignors to Crucible Steel Company of America, Pittsburgh, Pa., a corporation of New Jersey

Filed Dec. 27, 1966, Ser. No. 609,987  
11 Claims. (Cl. 75—214)

### ABSTRACT OF THE DISCLOSURE

This invention relates generally to the art of powder metallurgy and, more particularly, to a method for producing articles from powdered metal having large length to diameter ratios, whereby said articles may be further reduced to final thicknesses by the use of conventional rolling facilities. The method of the invention consists in the steps of placing a charge of powdered metal in an elongated tubular container, first compacting said container and charge by applying force in a direction normal to the axis of said container while preventing longitudinal extension thereof, second further compacting said container and charge by applying force in a direction normal to the plane of said first compacting force and the axis of said tubular container while longitudinal extension of the same is prevented, and finally compacting said container and charge to a final density of about 100 percent by simultaneously applying positive pressure at both ends of said container while the lateral spread thereof is restrained by a die. With the method described above, it is possible to produce from powdered metal, compacts suitable for rolling.

It is well known that by the use of powder metallurgy techniques, it is possible to produce metal articles, such as high-alloy steel articles, of fine grain size and homogeneous microstructure. The conventional practice for producing articles of this type is to place a charge of powdered metal of, for example, —100 mesh within a closed container that has been evacuated to a relatively low pressure, heat the container and charge of powdered metal to an elevated temperature of, for example, at least about 2000° F., compact the charge within the container by the application of suitable force while the charge is at elevated temperature, and finally remove the container from the compacted charge by machining, pickling or a combination of both. After removing the container from the compact, the compact may be either machined or forged to form the desired final product. Because of the extremely high pressures required to achieve compacting to a density of 100 percent, only relatively small compacts having low length to diameter ratios have been produced. Since, to permit rolling in conventional facilities, the workpiece must have a substantial length, for example at least about 42 inches, the working of compacts produced by powder metallurgy techniques to final products has been limited to forging and machining operations.

It is accordingly the primary object of this invention to provide a method for producing from powdered metal compacted articles having large length to diameter ratios, which enables them to be processed to final products by the use of conventional rolling facilities.

It is a further object of the invention to provide a method for producing from powdered metal compacted articles having large length to diameter ratios without requiring excessive total compacting pressures.

These and other objects of the invention, as well as a complete understanding thereof, may be obtained from the following description and drawings, in which:

2

FIGURE 1 is a perspective view of the elongated tubular container for the powdered metal to be compacted by the method of the invention;

FIGURE 2 is a diagrammatic showing of the first compacting step of the method;

FIGURE 3 is a transverse sectional view of the compact and container after the first compacting step of the method;

FIGURE 4 is a schematic view of the second compacting step of the method;

FIGURE 5 is a transverse sectional view of the compact and container after the second compacting step;

FIGURE 6 is a schematic showing of the final compacting step of the method;

FIGURE 7 is a perspective view of the final compact; and

FIGURE 8 is a schematic showing of final compact being subjected to a conventional rolling operation.

With reference to the drawings, in the practice of the method of the invention a charge of powdered metal, which has been thoroughly cleaned to remove surface oxides, is placed in a closed-end tubular container 10, as shown in FIGURE 1. The container is then connected by means not shown, to a vacuum pump, whereby the container interior is evacuated to a pressure of, for example, 50 microns or less. On evacuation, the container is heated to a temperature of at least, for example, 2000° F. Thereafter, the container 10 is placed within a die 12, as shown in FIGURE 2, and forces applied, as indicated by the arrows in FIGURE 2, to produce a compact having a cross section as shown in FIGURE 3. As may be seen in FIGURE 2, the container 10 is confined within the die 12 to prevent substantial longitudinal extension thereof during compacting. The compact is then placed within a die 14, as shown in FIGURE 4, and is further compacted by the application of force as indicated by the arrows in FIGURE 4 to produce a compact having a cross section as shown in FIGURE 5. During this compacting operation, the die prevents substantial longitudinal extension of the container. Thereafter, the compact, having a substantially square cross section as shown in FIGURE 5, is placed within a die 16, as shown in FIGURE 6, wherein the cross section of the die conforms substantially to that of the compact 10. Force is applied in the form of positive pressure simultaneously at both ends of the compact as indicated by the arrows in FIGURE 6. The die confines the compact during this operation and prevents the lateral spread thereof. By applying positive pressure simultaneously from both ends of the compact, the lateral forces during compacting are evenly distributed along the length of the compact. This results in a compact characterized by extremely uniform density from end to end. The final compact, as shown in FIGURE 7, after final compacting, as described above, has a density of about 100 percent. As also described above, its length to diameter ratio permits it to be processed as a conventional billet by the use of rolling facilities typically employed for billet rolling. Prior to this operation, the container 10 will be removed by acid pickling or machining. As shown in FIGURE 8, compact 10 is passed by means of conveyor rolls 17 longitudinally between a pair of horizontal work rolls 18, which in a conventional manner serve to reduce the compact to a desired final thickness. It is to be understood, of course, that during the above-described compacting operations, it is customary that the container and powdered metal charge therein are maintained at elevated temperature.

As a specific example, in the practice of the invention, a mild-steel pipe having a  $1/4$ -inch wall thickness, an inside diameter of 10 inches, and a length of about 50 inches was filled with a charge of —100 mesh AISIM2S steel powder. The container and charge of powdered metal were

heated to a temperature of approximately 2200° F. while the container was evacuated to a pressure of about 25 microns. Thereafter, the container and charge were subjected to initial compacting as described above with reference to FIGURE 2, to produce an intermediate compact having a width of approximately 12 inches and a thickness of about 6 inches. As described above, the longitudinal extension of the container was prevented during this compacting operation. During this initial compacting operation, the density of the charge was increased from an initial density of about 65 percent to a density of about 80 percent. Because of the low compacting densities required by this operation, compacting pressures of only 4 tons per square inch were required. The compact was then subjected to the second operation as shown in FIGURE 4 and described above, to achieve a compact of substantially square cross section of about 7½ inches. During this compacting step, the density of the compact was increased from the starting density of 80 percent to a density of about 95 percent. During this operation, pressures of about 4 tons per square inch were required. The compact was then placed on end within a die conforming substantially to the cross section of the compact along its entire length, and positive pressure, through the use of two rams, was simultaneously applied at both ends of the compact. By the application of pressure on the order of 20 tons per square inch, a final compact having a density of substantially 100 percent was achieved. The length of the final compact was about 47½ inches, which was suitable for subsequent reduction by the use of conventional billet-rolling facilities.

Examination of the compact after the final compacting step showed the same to have a substantially uniform density from end to end. This is caused by the extremely even distribution of lateral forces during the final compacting operation. Although, during the first two compacting operations pressure must be applied over a large surface area, the low pressures per unit area necessary to produce the relatively low intermediate densities required avoid the necessity for extremely high capacity presses. During the final compacting to the required final 100 percent density, extremely high pressures on the order of 20 tons per square inch are required; however, the surface area over which these high pressures must be applied is extremely small. Consequently, the requirement for extremely high capacity presses is again avoided.

During the practice of the invention as described above and shown in the drawings, during the first compacting operation, wherein compacting is achieved by applying force in a direction normal to the axis of the container, a compact density of at least about 80 percent is produced. During the second compacting step, wherein compacting forces applied in a direction normal to the plane of said first compacting force and the axis of said container, a density of at least about 95 percent is achieved. During final compacting, wherein compacting is achieved by simultaneously applying positive pressure at both ends of the container while the lateral spread thereof is restrained by a die, a density of substantially 100 percent is achieved. It is possible to eliminate the first compacting step by charging a container having a cross section as shown in FIGURE 3 with powder of a density permitting compacting to the desired final density by using only the second and final step as set forth above. During the entire compacting operation, the container and charge are, of course, at elevated temperature and at a pressure substantially less than atmospheric, preferably less than 25 microns, as described above. During the first two compacting steps, the longitudinal extension of the container and charge is, of course, prevented. For this purpose, the container is confined within a die during compacting. To facilitate processing of the final compact by conventional billet rolling facilities, a final compact having a substantially square cross section is preferred.

Although various embodiments of the invention have been shown and described above, it is obvious that other

modifications and adaptations may be made without departing from the scope and spirit of the appended claims.

What is claimed is:

1. A method for compacting metal powders to produce a compacted article having a length substantially greater than the cross sectional diameter thereof comprising placing a charge of powdered metal precompacted to a desired density and, to be further compacted into an elongated article, by placing said precompacted charge into a container, first compacting said charge by applying force in a direction normal to the axis of said elongated container, further compacting said charge by applying force axially to said elongated container, and removing said article from said container, said container being confined in a die during each compacting operation.
2. A method for compacting metal powders to produce a compacted article having a length substantially greater than the cross sectional diameter thereof comprising placing an uncompacted charge of powdered metal to be compacted into an elongated container, first compacting said charge by applying force in a direction normal to the axis of said elongated container, second further compacting said charge by applying force in a direction normal to the plane of said first compacting force and to the axis of said tubular container, further compacting said charge by applying force axially to said elongated container, and removing said article from said container, said container being confined in a die during each compacting operation.
3. A method according to claim 2 wherein the longitudinal extension of said charge and container is restrained by said die during compacting.
4. A method according to claim 2 wherein said charge during said second further compacting is compacted to a substantially square cross section.
5. A method according to claim 2 wherein said charge is compacted to a density of at least about 80 percent by said first compacting, to a density of at least about 95 percent by said second further compacting, and a density of substantially 100 percent by said final compacting.
6. A method according to claim 2 wherein said final compacting is effected by simultaneously applying positive pressure at both ends of said container while the lateral spread thereof is restrained by a die, whereby the resulting lateral forces are distributed substantially evenly along the length of said container.
7. A method according to claim 2 wherein said container is at elevated temperature and at a pressure substantially less than atmospheric during compacting thereof.
8. A method according to claim 7 wherein said container is at an elevated temperature of at least about 2,000° F.
9. A method according to claim 2 wherein the thickness of said article is reduced after final compacting by a rolling operation.
10. A method for compacting metal powders to produce a composite article having a length substantially greater than the cross sectional diameter thereof comprising placing a charge of powdered metal to be compacted into an elongated tubular container, first compacting said charge by applying force in a direction normal to the axis of said container, while the same is confined within a die, to a density of at least about 80 percent, second further compacting said charge by applying force in a direction normal to the plane of said first compacting force and the axis of said tubular container, while the same is confined within a die, to a density of at least about 95 percent, further compacting said charge to a density of about 100 percent by simultaneously applying positive pressure at both ends of said container while the lateral spread thereof is restrained by a die, whereby the resulting lateral forces are distributed substantially evenly along the length of said container, said container being at an elevated temperature of at least about 2,000° F. and at a pressure substantially less than atmospheric during compacting, removing said article from said container.

tainer, and reducing the thickness of said article by a rolling operation.

11. A method for compacting metal powders to produce a compacted article having a length substantially greater than the cross sectional diameter thereof comprising placing a charge of powdered metal to be compacted into an elongated container, first compacting said charge by applying force in a direction normal to the axis of said elongated container while substantially restricting the longitudinal extension thereof, further compacting said charge by simultaneously applying positive pressure at both ends of said container while the lateral spread thereof is restrained by a die, whereby the resulting lateral forces are distributed substantially evenly along the length

of said container, removing said article from said container, and reducing the thickness of said article by a rolling operation.

**References Cited****UNITED STATES PATENTS**

2,386,604 10/1945 Goetzel ----- 75-214 X  
3,075,244 1/1963 Glenn ----- 75-214 X

**FOREIGN PATENTS**

638,609 3/1962 Canada.

BENJAMIN R. PADGETT, *Primary Examiner.*

A. J. STEINER, *Assistant Examiner.*